

## UNITED STATES PATENT OFFICE

GEORGE E. KENDALL, OF KALAMAZOO, MICHIGAN

## METHOD OF MANUFACTURING ARTIFICIAL STONE

No Drawing.

Application filed March 5, 1926. Serial No. 92,636.

The object of this invention is to provide an improved method and process of manufacture which will secure an artificial stone with very dense smooth surface having the 5 appearance of being polished in imitation of marble or any other cut face and polished stone, and the improved product which may imitate marble or granite.

Objects pertaining to details will appear 10 from the detailed description to follow. The invention is defined in the claims.

My improved method or process consists in providing a mold with a face plate for 15 making the face of the stone which is impervious to moisture and smooth. This may be a glass sheet or sheet metal or any other material. I then apply to the face plate a mixture of Portland cement, preferably one part cement to one part sand, using an excessive amount of water far beyond what is 20 necessary to set the cement. I mix the same and stir it so that it is of a paint-like consistency, with all colloids fully developed, and apply it to the smooth face of the mold 25 with a brush, thoroughly working it into contact with the said face, and placing the mold face plate down so that none of the moisture will drain off.

If it is desired to produce patterns in the 30 stone in imitation of marble or other irregularity, I apply the pattern to this painted coating on the back side, forcing it through the layer with a blunt pointed implement so that it penetrates to the face of the mold, 35 leaving a characteristic colored mark, applying in this way any coloring matter. Of course, to secure the most permanent results a mineral pigment is required.

When the surface has been thus prepared, 40 I fill the balance of the mold with a grout, preferably of four parts sand to one part cement, making it very wet so that it pours. As soon as this has partially set, or immediately if that is expedient, I place the mold 45 face down so that it will accumulate water on the face plate in excess of that needed for the setting of the cement. I then cover the whole with damp sand of sufficient volume and thickness, or otherwise protect 50 the same, to prevent evaporation of the

moisture, retaining the same and allowing the cement to set, preferably for a period of not less than ten days. A shorter period secures only fair results and perfect results are not secured under ten days. At the end of 55 that time I remove the block from the mold. It is necessary to start at one edge of the face plate and open it very carefully to admit air, which causes the film of water to divide and separate, leaving a surface which is as 60 smooth as ordinary polished marble. This surface must not be touched because it is likely to abrade until it has become dry and hard.

When this surface is completed it does not 65 appear to be of a crystalline character, but amorphous or waxy, as it can be readily dented without breaking. The kind of Portland cement used is not material, so far as I have observed. If imitation marble is desired, I use white cement. If granite is desired, I use the ordinary gray cement. Either of these can be colored as desired and with any suitable design. A very effective 70 plain stone is secured without injecting in the 75 design.

I wish to claim the invention broadly and specifically, and also the design and the coloring in the manner described, because the effect is very similar to the effect of natural 80 marble or stone.

Having thus described my invention, what I claim as new and desire to secure by Letters Patent is:

1. The process of making artificial marble 85 or stone consisting in providing a mold with a face plate of flat, smooth, impervious, waterproof material, applying thereto with the face plate down a rich paint-like, wet mixture of cement with a brush to develop 90 the colloids and completely and closely cover the surface, injecting through the mixture suitable color designs by scratching with a blunt pointed instrument, thereafter covering the whole with grout of substantially 95 four parts sand to one part cement, wetting the same thoroughly, placing the mold with face plate down, and covering the whole with damp sand to retain the moisture, allowing it to stand a sufficient time to fully 100

set, then removing it from the mold, and separating the face plate from one edge carefully to insure the separation due to the film of water formed between the face plate and the stone, as specified.

5 2. The process of making artificial marble or stone consisting in providing a mold with a face plate or flat, smooth, impervious, waterproof material, applying thereto with  
10 the face plate down a rich, paint-like, wet mixture of cement with a brush to develop the colloids and completely and closely cover the surface, thereafter covering the whole with grout of substantially four parts sand  
15 to one part cement, wetting the same thoroughly, placing the mold with face plate down, and covering the whole with damp sand to retain the moisture, allowing the same to stand a sufficient time to fully set,  
20 then removing it from the mold, and separating the face plate from one edge carefully to insure the separation due to the film of water formed between the face plate and the stone, as specified.

25 In witness whereof I have hereunto set  
my hand.

GEORGE E. KENDALL.

30

35

40

45

50

55

60

65